

1

2,895,821

**PROCESS FOR REFINING BLISTER COPPER.**

Eugene R. Redmond, Oracle, Ariz., assignor to Brian Jackson Associates Inc., Tucson, Ariz., a corporation of Arizona

No Drawing. Application May 18, 1954  
Serial No. 430,725

3 Claims. (Cl. 75—75)

This invention relates to improvements in the refining of copper and more particularly to the refining of blister copper to produce flat copper.

As conventionally practiced, the refining of copper involves three major steps, namely, first, the production of copper matte in a reverberatory furnace; second, the treatment of copper matte in a converter furnace to produce "blister" copper; and third, the further treatment of "blister" copper either by fire refining or electrolytic refining to produce a marketable product. The second step, wherein the iron and sulphur present in copper matte are oxidized and removed to leave blister copper as an end product, is known in the copper smelting trade as "converting."

Converting of copper matte is essentially divided into two parts, the first part being the "slagging" period during which, as air is blown into the molten matte, the iron is oxidized and combines with added siliceous flux to form a slag which is readily removed leaving a molten mass of copper bearing material consisting principally of copper sulphide. The second part is the "finish" period during which air is again blown into the molten material, usually at an elevated temperature of about 2200° F., resulting in the oxidation of the copper sulphide to yield metallic copper and sulphur dioxide.

When the copper sulphide has been substantially all oxidized the blow is stopped and the resulting or end product, known in the trade as blister copper, is transferred to a fire refinery or electrolytic furnace for further purifying and refining.

In such further purifying and refining treatment, whether by fire refining or electrolytic refining, it is necessary that the blister copper be further oxidized until at least saturated with copper oxide, whereupon the blow is usually stopped, the accumulated slag skimmed off, and the copper subsequently reduced and cast.

The process of the present invention departs from present conventional practice in that the further purifying and refining of "blister" copper, and the saturation thereof with copper oxide, is carried out in the converter in a fraction of the time previously required and without the necessity of transferring the materials to a separate furnace for such further treatment. Moreover, such further treatment may be accomplished at temperatures somewhat lower than those required in the production of blister copper and without the formation of a copper oxide slag, which is harmful to the converter linings.

In practicing the present invention, the refining of copper may be carried out in the conventional manner described above up to and including the production of blister copper in the converter. Customarily, the process would be stopped here, the material poured out of the converter and transferred to another furnace for further treatment. However, in accordance with the present invention the blowing of the material is continued beyond the blister stage to and through the worm stage, preferably at a slightly reduced temperature. This further blowing and oxidation of the material is continued until

2

the "worm" is about to leave the copper, at which time the copper is substantially saturated with copper oxide. At this point a silica flux of the usual or any well known type for the purpose is added to the material in the converter and the blow continued, preferably at a temperature in the neighborhood of about 2150° F. until the copper is substantially free of impurities. The converter is then turned out and the blow terminated. The resulting product is highly refined copper comparable in every way to the product obtained by fire refining which, as previously indicated herein, is conventionally accomplished in a separate furnace particularly designed for the purpose.

The addition of the silica flux to the material just as the worm is beginning to disappear is an important feature of the invention in that it causes the granulated slag, formed during such further blowing of the copper past the "blister" stage and containing the principal impurities of "blister" copper, to form a coating, which allows the copper to be withdrawn, leaving the impurities in such coating. Such coating, moreover, contains little, if any, copper or copper oxide, and thence need not be used as a recirculating load in the converters.

The particular point at which to add the silica flux can be determined by taking samples of the material as it is blown through the worm stage. Thus, as the blowing is continued and successive samples are taken, it will be noted that the "worm" becomes smaller and smaller and eventually disappears. This is referred to in the trade as "blowing the worm off the copper." Just as the worm is about to disappear, which may readily be determined by one skilled in the art, the silica flux is added.

An alternative and commercially preferred manner of determining the proper time to add the silica flux is based on observation of the sparks in the gas stream leaving the converter. Thus, it has been found that when the blow has progressed to the point where the "worm" is just about to disappear, the sparks in the gas stream from the converter begin to appear to break or burst whereupon the silica flux is added as before.

Following addition of the flux, the blow is continued until the copper is substantially free of impurities. The particular time required for this phase of the treatment will depend, of course, on the size of the charge, the blowing rate, and the exactness with which the point of addition of the flux was determined. As an example, where the charge is about 75 to 80 tons of the molten mass to which has been added about 2½ tons of silica or quartz flux, the time required will be approximately 5 minutes. This may be varied, however, to suit the particular conditions of treatment.

The point at which the blow is to be stopped and the treatment terminated may be determined by sampling, as before, or alternatively, by observing the characteristics of the gases leaving the converter. Thus, as the blowing is continued, following addition of the flux, it has been found that the gaseous flames leaving the converter become noticeably more transparent until a point is finally reached when the flame becomes almost completely transparent. It is at this point that the copper is substantially free of impurities whereupon the converter should be turned out and the blow terminated.

The silica flux added may be of the type commonly used for the production of blister copper. The amount to be added, will vary, of course, with the particular material and the conditions of treatment. In general, however, it has been found that satisfactory results are obtained if the added flux constitutes from about 2 to about 5 percent, by weight, of the charge.

The temperatures employed in the further refining of blister copper in accordance with the process of the in-

vention need not be higher than those employed in the production of blister copper and will usually be somewhat lower. Thus the temperatures employed at the start of the blow, i.e., after the formation of the blister copper, will generally not exceed about 2250° F. and will usually be somewhat lower as, for example, from about 2150° F. to about 2200° F. As the blow progresses temperatures may be further reduced and it is possible to finish the copper at a temperature as low as about 2050° F.

The process herein disclosed is to be distinguished from a practice sometimes employed in smelters where copper anodes are to be cast as part of the process, namely, the practice of blowing the copper past the blister stage at increased temperatures to oxidize the slag and remove more of the small traces of iron and other impurities remaining in the copper. The gain by doing this is a reduction in the time of lance blowing necessary in the anode furnace itself to remove these impurities. However, due to the high temperatures required, which sometimes run as high as 2600° F., a substantial amount of copper is lost in the slag and thus the slag must be skimmed off and rehandled as a circulating load in the converters. These high temperatures, moreover, quickly burn out the brick linings of the converters making frequent replacements necessary, and finally, the resulting copper must still be blown in the anode furnace for an appreciable time to remove impurities.

In the process of the present invention, on the other hand, the temperatures employed do not exceed those used in the production of blister copper and are usually somewhat lower. Moreover, the addition of the flux as the worm is about to disappear causes the formation of a coating permitting the copper to be removed and leaving the impurities in the coating.

The process of the present invention represents a complete departure from the conventional methods of refining copper. It makes possible the further refining of blister copper directly in the converter without the necessity of transferring the blister copper to a separate furnace for further treatment. Moreover, such further refining of blister copper is accomplished in a fraction of the time required in conventional practice thereby permitting increased production and more economical production.

As herein used, the term "blister" copper refers to a product which is essentially free of copper sulphide, and contains 98 percent or more copper by weight, the principal impurities being iron, sulphur, and oxygen. On cooling, blister copper solidifies with a surface covered with "craters" or "blisters." If a section is cut through this copper, it is found to be porous.

The term "worm" copper, as herein used, refers to a product which contains more copper oxide than blister copper. In other words, it is copper which has been carried further along in the oxidizing process. A sample of "worm copper" on cooling first solidifies over the top

and then the molten copper, under pressure of the contained gases, breaks through the solid layer and runs over it as a worm might crawl. This is commonly spoken of as "throwing a worm." As previously indicated herein, if samples are taken of copper as it is blown beyond the worm stage, it is seen that the "worm" becomes smaller and smaller as the blowing is continued and eventually disappears.

The term "flat copper," as herein used, refers to a purified product obtained for example, by the fire refining of "blister" copper, or by the further refining of blister copper in accordance with the process herein disclosed.

While the process of the invention has been described in some detail the scope of the invention is not to be construed as limited thereby otherwise than as covered in the following claims.

I claim:

1. In the process of refining blister copper in the converter in which it is formed which includes blowing air into a molten mass of blister copper, and continuing the air blow to the worm stage, the improvement comprising refining said blister copper through the worm stage including the steps of adding a silica flux to the mass as the worm is just about to disappear, continuing the blow until the silica flux has formed a solid coating over said mass and pouring said mass out from under said coating.

2. In a process of refining blister copper containing free sulfur in the converter in which it is formed which includes blowing air into a molten mass of blister copper, and continuing the blow until the copper is substantially free of said sulfur, the improvement comprising adding a silica flux to the molten mass of material, and continuing the air blow at a temperature not in excess of about 2150° F. until the silica absorbs said free sulfur and solidifies, and pouring the copper out from under said solidified silica.

3. A process of refining blister copper in the converter in which it is formed which comprises air blowing the same to and through the worm stage at a temperature between about 2050° F. and 2250° F., adding a silica flux to the molten mass of material when the sparks therefrom begin to have the appearance of breaking or bursting, and continuing the air blow until the gaseous flames from the molten mass are substantially completely transparent.

#### References Cited in the file of this patent

#### UNITED STATES PATENTS

50 723,500 Thofehrn et al. ----- Mar. 24, 1903

#### FOREIGN PATENTS

472,626 Great Britain ----- Sept. 23, 1937

#### OTHER REFERENCES

Newton: Metallurgy of Copper, pages 196, 197, 202, 1942.